

## UNITED STATES PATENT OFFICE

2,318,710

## GUM INHIBITOR

Albert A. Persyn, Associated, Calif., assignor to  
 Tide Water Associated Oil Company, San Fran-  
 cisco, Calif., a corporation of Delaware

No Drawing. Application February 12, 1940,  
 Serial No. 318,589

2 Claims. (Cl. 196—150)

This invention relates to the prevention or suppression of the formation of gum in cracked, polymerized, and similar gasolines and has for a principal object the addition of a particular inhibiting agent to gasolines which normally tend to form gum.

Various means have been employed for the suppression of the formation of gum in cracked gasolines, polymer gasolines, and gasolines obtained from other pyrolytic processes.

These methods generally consist in adding to the gasolines small percentages of various substances which apparently have a selective affinity for oxygen, thus preventing the oxygen from combining with the more reactive constituents of the gasoline to form resinous material, or gum, which would form troublesome deposits in various parts of the gasoline engine during use.

Most inhibitors in general use are somewhat, if not readily, soluble in water. To be entirely satisfactory as an inhibitor a material should be practically water insoluble to prevent its being extracted from the gasoline by any water with which the gasoline may come in contact during storage. It is, therefore, an object of this invention to provide an inhibitor which is water insoluble.

It has been found that the extract obtained when treating straight run distillates with a selective solvent such as, for example, with liquid sulphur dioxide, aniline, acetonitrile, etc. has good gum-inhibiting properties when mixed with cracked or polymer gasoline.

For this purpose, and according to the invention, there is added to a cracked gasoline, or other gasoline, which normally would tend to form gum in storage, about 5% of a selective solvent extract obtained from a straight run distillate. The particular percentage added depends upon the amount of inhibiting property desired and may range from 1% to about 10% or more.

The particular boiling range of the extract is important. It has been found that the higher the boiling range the better is the inhibiting property. However, too high a boiling range is to be avoided as this will increase the end boiling point of the gasoline depending on the amount used. The preferred boiling range of the extract is between about 350° to 450° F., although 300° F. to 500° F. or higher, or lower, may be used.

Methods for the preparation of the selective solvent extract are well known in the art. Briefly stated they involve treating a straight run distillate with about 100% to 300% by volume of a selective solvent, such as liquid sulphur dioxide

for example. The selective solvent dissolves the more aromatic constituents and, after separation of the solvent layer, the solvent is evaporated leaving the dissolved constituents as extract. Such extracts have been used as a means for supplying high anti-knock constituents to an otherwise low octane rating gasoline, such as straight run gasoline. For such purposes rather large quantities of the extract are needed. For instance three parts of a gasoline having 60 octane rating will require one part of the extract to raise the octane rating to about 65.

In contradistinction to the use of selective solvent extracts for increasing the antiknock quality of gasolines, the present invention contemplates the addition of much smaller amounts (less than 10% in most cases) of the extract to a gasoline which is already rather high in antiknock rating. As cracked gasolines and polymer gasolines normally have octane ratings of 70 or higher, it will be readily appreciated that the addition of from 5% to 10% of extract, with an octane rating of about 80, will not appreciably affect the octane rating of the blend.

It is further to be noted that straight run gasolines, to which such extracts are customarily blended, are gum stable and have no appreciable tendency to form gum. It is thus seen that the addition of the extract to cracked and polymer gasolines, which normally tend to form gum, performs a novel function not contemplated when the extract is blended with straight run gasoline.

The following are examples of the effectiveness of the extract to suppress the formation of gum in cracked and polymer gasoline:

## EXAMPLE I

A mixture of nine parts light cracked gasoline and one part of polymer gasoline and having a distilling range of 100° F. to 380° F. was blended with various amounts of a straight run extract having a distilling range of about 350° F. to 450° F. The various blends were then tested for stability in accordance with the test described in an article entitled "Inhibitors in cracked gasoline" published in Industrial and Engineering Chemistry, volume 24 (1932), pages 1375 to 1382. The method consists briefly in sealing a sample of the gasoline in a steel bomb under 100 pounds gage pressure of oxygen and heating for several hours at a temperature of 212° F. The length of time of heating until there is a sharp reduction in the oxygen pressure (due to oxidation reactions in the gasoline) is called the "induction period" and is generally

recognized in the art to be indicative of the gum stability of the gasoline under test. Table I shows the induction period of the gasoline with and without extract.

Table I

| Blend                          | Induction period |
|--------------------------------|------------------|
|                                | Minutes          |
| 100% basic gasoline blend      | 20               |
| 98% basic gasoline+2% extract  | 80               |
| 95% basic gasoline+5% extract  | 395              |
| 90% basic gasoline+10% extract | 900              |

## EXAMPLE II

A similar blend of cracked and polymer gasolines were blended with straight run extract as before. Table II shows the induction period of the blends.

Table II

| Blend                          | Octane No. | Induction period |
|--------------------------------|------------|------------------|
|                                |            | Minutes          |
| 100% basic gasoline blend      | 78         | 45               |
| 95% basic gasoline+5% extract  | 78         | 240              |
| 90% basic gasoline+10% extract | 78.5       | 450              |
| 85% basic gasoline+15% extract | 78.5       | 540              |

The term "gasoline" as used herein is intended to mean any fuel suitable for a carbureted internal combustion engine and composed principally of hydrocarbons. The preferred boiling range preferably lies within that commonly used for such purposes, i. e. 80° F. to 437° F. However, cracked gasolines with distillation end points of 350° to 380° F. are commonly used. Gasolines with higher end points than 437° F. may be used.

The term "selective solvent extract" is used to denote the more aromatic constituents of petroleum which are dissolved in selective solvents of the type exemplified by liquid sulphur diox-

ide, aniline, and acetonitrile. A number of these solvents are known and used in the art to dissolve and separate the more aromatic constituents of petroleum from the more paraffinic constituents. By far the most suitable of these solvents for the present purposes is liquid sulphur dioxide, due to its low boiling point and consequent ease of separation from the extracted material.

- 10 I claim:
1. The process of suppressing the formation of gum in cracked, polymerized, and other pyrolytic gasolines intended for use as fuel for an internal combustion engine and of the type tending to deposit gum during storage, which consists in removing such gum inhibitor compounds from straight run petroleum fractions within the boiling range 350°-450° F. by treatment with a selective solvent of the type which dissolves the more aromatic hydrocarbons and other compounds, and adding the selective solvent extract to such gasoline in an amount between 2% and 10% of the gasoline, thereby the octane number of the gasoline is not materially altered but the time of formation of gum in the gasoline during storage is greatly lengthened, said extract boiling at temperatures below 450° F. and hence being volatile when carbureted in the internal combustion engine.
  - 15 2. A motor fuel comprising a cracked gasoline of the type normally tending to deposit gum during storage, and from 2% to 10% of a selective solvent extract from a straight run petroleum distillate within the boiling range 350°-450° F., said extract containing gum inhibiting compounds to delay the formation of gums in cracked gasoline, and being in the boiling range of the cracked gasoline, and said motor fuel having approximately the same octane number as
  - 20 25 30 35 40 the cracked gasoline alone.

ALBERT A. PERSYN.